

Aug. 4, 1953

N. E. COOK ET AL.

2,647,304

## PROCESS OF TERNE COATING METAL AND TERNE COATED PRODUCT

Filed Aug. 18, 1951

*Fig. I.*



*Fig. 2.*



## INVENTORS

**NELSON E. COOK &  
SAMUEL L. NORTEMAN**

SAMUEL L. NORTEMAN  
by George, Lewis & Tolman  
his attorneys

## UNITED STATES PATENT OFFICE

2,647,304

PROCESS OF TERNE COATING METAL AND  
TERNE COATED PRODUCT

Nelson E. Cook and Samuel L. Norteman, Wheeling, W. Va., assignors to Wheeling Steel Corporation, Wheeling, W. Va., a corporation of Delaware

Application August 18, 1951, Serial No. 242,496

3 Claims. (Cl. 29—194)

1

This invention relates to the terne coating of metal and to an improved terne coated product. It relates particularly to an improvement in the manner of heating a bath of molten terne metal employed for hot dip terne coating whereby improved improved results are obtained.

Terne metal comprises lead and tin with lead in preponderance. Normally the percentage of tin is between about fifteen per cent. and somewhat over twenty per cent.; the remainder is substantially all lead except for impurities.

In the hot dip terne coating of metal the metal to be coated is first immersed in a flux bath, commonly zinc chloride, after which the metal being coated is immersed in a bath of molten terne metal in a pot. Prior to our invention the pot has been heated externally to maintain the bath of terne metal molten. Normally the surface of the bath of molten terne metal is divided by a partition member and a bath of oil, usually palm oil or a combination of palm and mineral oils, is floated upon the bath of molten terne metal at one side of the partition member. The metal to be coated is introduced into the bath of molten terne metal at the side of the partition member opposite the side at which the oil bath floating upon the terne metal is disposed. The metal being coated passes through the bath of molten terne metal beneath the partition member and emerges through the oil bath. The use of such an oil bath is well known in the art, the oil acting on the terne metal adhering to the metal being coated to produce a terne coating thereon which is continuous, smooth and desirably free from "pin holes."

Optimum results are obtained when the oil of the oil bath has a relatively low flash point. However, the flash point of the oil must be above the temperature of the bath of molten terne metal as otherwise the oil will ignite and burn. Despite efforts to avoid igniting the oil there have been many occurrences of oil ignition in terne coating pots, some of which have resulted in injuries, serious fires and great damage.

Since it is desirable that the flash point of the oil employed to form the oil bath floating upon the bath of molten terne metal be as low as practicable, the efforts of those skilled in the art have been directed to maintaining as small a difference between the temperature of the bath of molten terne metal and the flash point of the oil as is consistent with safety. The minimum permissible flash point of the oil has been limited by so-called "hot spots" or localized zones of undesirably high temperature in the molten terne

2

metal which have unavoidably occurred due to the application of heat to the terne metal through the coating pot. It has been necessary to use an oil which will not flash when subjected to the relatively high temperatures encountered at hot spots, and since the maximum temperatures at hot spots are uncertain the application of the necessary factor of safety has resulted in inability to employ oil of desirably low flash point. Despite precautions injuries, serious fires and great damage have occurred and will continue to occur when externally heated terne coating pots are employed.

It is desirable for several reasons to employ a relatively high proportion of tin in the terne metal. The tin aids in bonding the terne metal to the metal being coated, contributes to a sound strong bond, renders the coating desirably fluid as it is applied to the metal being coated and minimizes "pin holing" which is one of the most common defects in terne coatings. Moreover, tin has a much lower melting point than lead, so the greater the proportion of tin in the terne metal the lower will be the melting point of the terne metal and consequently the lower may be the temperature of the bath of molten terne metal and the lower may be the flash point of the oil forming the oil bath floating on the bath of molten terne metal.

Normally tin is incorporated in terne metal to between fifteen and twenty-two per cent. A rule of thumb as to the composition of terne metal is that it contains four parts of lead to one part of tin. However, tin is relatively scarce

and difficultly obtainable and for economic reasons it is necessary to reduce the proportion of tin in terne metal to an undesirably low proportion. At the present time government restrictions limit the proportion of tin which may be

used in terne metal to ten per cent. One of the most serious disadvantages of the limitation of the proportion of tin in terne metal is that the temperature of the bath of molten terne metal of necessity becomes undesirably high since the temperature of any molten bath is determined by the melting point of the material of which the bath is constituted. This means that the flash point of the oil employed to form the oil bath floating upon the bath of molten terne metal

must likewise be undesirably increased. The results are difficulty of operation, the production of an inferior product and increased danger of fire unless at the higher temperatures employed the factor of safety as applied to temperature differential between the bath of molten terne

metal and the oil bath floating on the bath of molten terne metal is increased, which further detrimentally affects the process and product.

We have discovered how to obviate the disadvantages above referred to, which disadvantages are real and serious and exist today in all externally heated terne coating pots. We provide for maintaining the terne metal molten by electric induction heating and thereby maintaining the temperature of the terne metal substantially uniform throughout the bath of molten terne metal and substantially eliminating hot spots. This makes it feasible to use oil having a materially lower flash point than could be used with an externally heated terne coating pot with the attendant advantages above indicated in the coating procedure and improved quality of the product produced. Moreover, because of the relatively uniform temperature of the molten terne metal insured by the use of electric induction heating it is possible without sacrifice of safety to reduce somewhat the differential between the temperature of the molten terne metal and the flash point of the oil employed. The use of electric induction heating results in maintenance of the molten terne metal at a remarkably constant temperature with the result that a product of unprecedentedly uniform superior quality is produced without incurring any more danger of fire than is incurred in the use of externally heated terne coating pots; indeed, the danger of fire is less even while the improved results are obtained.

Other details, objects and advantages of the invention will become apparent as the following description of a present preferred method of practicing the same and of apparatus upon which the invention may be practiced proceeds.

In the accompanying drawings we have shown apparatus upon which our invention may be practiced and have illustrated a present preferred method of practicing the invention in which

Figure 1 is a central vertical longitudinal cross-sectional view, taken on the line I—I of Figure 2, of hot dip terne coating apparatus for coating strip; and

Figure 2 is a cross-sectional view of the apparatus shown in Figure 1 taken on the line II—II of that figure.

Referring now more particularly to the drawings, there is shown apparatus for terne coating strip. Similar apparatus except modified as to the means used for passing the work through the pot may be used for terne coating articles. Since our invention does not lie in the means for passing the work through the pot the terne coating of strip is illustrated purely by way of example, the method so far as the invention is concerned being the same when articles are coated.

The strip being coated is designated 2 and the pot is designated generally by reference numeral 3. The strip is guided for movement through the pot by guide rolls 4, 5 and 6, conventional exit rolls 7 as known to those skilled in the art being employed in the usual manner.

As the strip 2 enters the pot 3 it passes through a flux box 8 which may be of conventional structure containing a bath of flux, such as zinc chloride. The strip before passing through the flux is desirably pretreated and washed as known to those skilled in the art.

The strip after passing through the flux in the flux box 8 is immersed in a bath 9 of molten

terne metal contained in the pot 3. The pot 3 is supported by a framework 10 and comprises an outer metal shell 11, a lining 12 of insulating material and a refractory inner lining 13 for containing the bath of molten terne metal 9.

We provide on the pot 3 one or more lateral extensions (two opposed extensions being shown) each designated generally by reference numeral 14. Each extension 14 comprises a refractory lining 15 communicating with the refractory lining 13 of the pot proper and which forms a passage 16 which extends laterally and downwardly from a side of the pot. Each passage 16 communicates with the interior of the pot at the upper portion thereof as shown in Figure 1 and extends outwardly and downwardly. The cross section of each passage 16 preferably decreases from relatively great cross section inwardly of the pot to relatively small cross section outwardly of the pot. Each passage 16 communicates with three outwardly and downwardly directed ducts 17 which at their outer extremities enter a cross duct 18. Disposed in a closed loop about the central one of the three ducts 17 is a magnetic core 19 having formed on each of the legs thereof extending between the central duct 17 and an outer duct 17 a coil 20 to which electric current is conducted. The current conducted to the coils 20 may, for example, be 440 volt, single phase, 60 cycle alternating current. There may be provided a pack of static capacitors for power factor correction, contactors for switching from high to low voltage for temperature control, a circuit breaker and auxiliary equipment for automatic control of power input to maintain a desired temperature in the body of the molten terne metal 9.

A low voltage is induced across the ducts 17. The apparatus is analogous to a step-down transformer having a short-circuited secondary which is formed by molten metal filling the ducts 17 and 18. Since the ducts 17 and 18 form a closed circuit a current will flow in them. The current generates heat in the terne metal itself which is the heat maintaining the bath of terne metal molten.

The heat generated in the metal causes a continuous and rapid thermal circulation of the molten terne metal across the pot which maintains the bath of molten terne metal at substantially uniform temperature throughout the bath. It inhibits the formation of hot spots in the bath and enables regulation of the bath temperature to an extent impossible when the pot is heated externally. Because of the close regulation and maintenance of a substantially uniform temperature throughout the bath of molten terne metal we are enabled to use with safety on the surface of the molten terne metal an oil having a much lower flash point than could be used otherwise with a significant improvement in the quality of the coated product.

A partition member 21 extends across the pot substantially at right angles to the axis of the pot which joins the two passages 16 so as to intersect the surface of the bath of molten terne metal 9, the bottom of the partition member 21 being disposed somewhat below the surface of the molten terne metal. The strip 2 is immersed in the molten terne metal 9, being introduced thereinto to the left of the partition member 21 viewing Figure 1. The strip passes beneath the partition member 21 and after passing about the guide roll 5 and between the exit rolls 7 is withdrawn from the pot to the right of the partition

member 21 viewing Figure 1. Disposed atop or floating upon the bath of molten terne metal to the right of the partition member 21 viewing Figure 1 is a bath of oil 22, which is the bath of oil above referred to and which has a flash point somewhat higher than the temperature of the bath 9. The bath 9 is substantially free from hot spots so there is no danger of igniting the oil bath 22 through localized increase of its temperature to or above the flash point of the oil. The heating of the bath of molten terne metal by electric induction heating also results in longer pot life and the formation of less scruff. Scruff is formed by deterioration of the pot by the molten terne metal, and we inhibit such deterioration. Moreover, the heating of the bath of molten terne metal by electric induction heating results in superior mixing of the constituent metals and inhibits settling out of the lighter metal on top of the heavier metal. These factors further contribute to a greatly improved product and the obtaining of optimum conditions with a uniformity and regularity not possible with an externally heated pot.

The specific gravity of the molten terne metal 9 is, of course, very much higher than the specific gravity of either the flux in the flux box 8 or the oil 22. The flux is designated 23, its upper surface in the flux box being shown at 24. The level of the molten terne metal 9 to the left of the partition member 21 viewing Figure 1 and outside the flux box is shown at 25 while the level of the molten terne metal 9 within the flux box where the weight of the flux is superimposed upon it is shown at 26. The surface of the oil 22 is shown at 27 and the surface of the molten terne metal 9 to the right of the partition member 21 where the oil 22 is superimposed upon the molten terne metal is shown at 28.

While we have illustrated and described a present preferred method of practicing the invention it is to be distinctly understood that the invention is not limited thereto but may be otherwise variously practiced within the scope of the following claims.

We claim:

1. In the terne coating of metal in which metal is immersed in a bath of molten terne metal and removed from the bath of molten terne metal through a bath of oil floating atop a portion

of the bath of molten terne metal and in which the temperature of the molten terne metal approaches the flash point of the oil so that there is danger of igniting the oil by so-called "hot spots" or localized zones of undesirably high temperature in the molten terne metal, the step of maintaining the terne metal molten by electric induction heating and thereby maintaining the temperature of the terne metal substantially uniform throughout the bath of molten terne metal and substantially eliminating "hot spots" whereby to obviate the danger of igniting the oil.

2. In the terne coating of metal in which metal is immersed in a bath of molten terne metal containing not over about 10% tin with the remainder being substantially all lead except for impurities and the metal being coated is removed from the bath of molten terne metal through a bath of oil floating atop a portion of the bath of molten terne metal and in which the temperature of the molten terne metal by reason of the presence of an undesirably small proportion of relatively low melting point tin and an undesirably great proportion of high melting point lead is higher than optimum terne coating temperature and approaches the flash point of the oil so that there is danger of igniting the oil by so-called "hot spots" or localized zones of undesirably high temperature in the molten terne metal, the step of maintaining the terne metal molten by electric induction heating and thereby maintaining the temperature of the terne metal substantially uniform throughout the bath of molten terne metal and substantially eliminating "hot spots" whereby to obviate the danger of igniting the oil.

3. A terne coated product comprising a base metal having thereon a coating of terne metal of improved uniformity and quality applied by the process of claim 1.

NELSON E. COOK.  
SAMUEL L. NORTEMAN.

References Cited in the file of this patent

UNITED STATES PATENTS

| Number    | Name             | Date          |
|-----------|------------------|---------------|
| 2,108,381 | McElhaney et al. | Feb. 15, 1938 |
| 2,520,349 | Tama             | Aug. 29, 1950 |